

# United States Patent [19]

Sherwood et al.

[11] 4,347,063

[45] Aug. 31, 1982

[54] PROCESS FOR CATALYTICALLY GASIFYING CARBON

[75] Inventors: Rexford D. Sherwood, Suffern, N.Y.; Rees T. K. Baker, Murray Hill, N.J.; Eric G. Derouane, Champion, Belgium; Wim J. Pieters, Morristown, N.J.

[73] Assignee: Exxon Research & Engineering Co., Florham Park, N.J.

[21] Appl. No.: 248,266

[22] Filed: Mar. 27, 1981

[51] Int. Cl.<sup>3</sup> ..... C10J 3/00

[52] U.S. Cl. ..... 48/197 R; 252/312; 585/733

[58] Field of Search ..... 48/197 R; 252/372; 585/733

## [56] References Cited

### U.S. PATENT DOCUMENTS

4,005,995 2/1977 Tamai et al. ..... 48/197 R  
4,242,103 12/1980 Rabo et al. ..... 585/733

### OTHER PUBLICATIONS

Keep et al., "Studies of the Nickel-Catalyzed Hydrogenation of Graphite", Journal of Catalysis 66, pp. 451-462, (Dec. 1980).

Primary Examiner—Peter F. Kratz  
Attorney, Agent, or Firm—Edward M. Corcoran

## [57] ABSTRACT

Carbon is gasified with steam in the presence of a catalytic metal such as nickel by forming a dispersion of the metal on graphite wherein the average particle size of the dispersed metal is below about 100 Å and preferably below 25 Å in diameter and contacting the dispersed metal/graphite composite with steam at about 800° C. or higher to gasify the graphite. This process will also gasify mixtures of graphite and amorphous carbon.

9 Claims, 3 Drawing Figures





FIG. 1



FIG. 2

FIG. 3

Relationship between Nickel particle size and  
channel propagation rate in steam at 1000°C



PROCESS FOR CATALYTICALLY GASIFYING  
CARBON

BACKGROUND OF THE INVENTION

1. Field of the Invention

This invention relates to gasifying carbon. More particularly this invention relates to catalytically gasifying carbon with steam. Still more particularly, this invention relates to catalytically gasifying carbon with steam in the presence of a catalytic metal such as nickel by forming a dispersion of such metal on graphite as particles below about 100 Å in diameter and contacting said metal/graphite composite with steam at a temperature of at least about 800° C. to gasify the carbon.

2. Background of the Disclosure

Metals of Groups VIB and VIII of the Periodic Table, such as Ni, Co, Mo and mixtures thereof, are known to be useful for catalytically gasifying carbon with steam and/or hydrogen. Those skilled in the art know that when depositing such metal on graphite or when forming a metal/graphite composite, the average particle size of the catalytic metal on a graphite support generally ranges from about 50 Å to 1,000 Å in diameter, with the vast majority of such catalysts having particles whose average diameters range from between about 50 Å to 250 Å and generally above about 100 Å. Another problem associated with the use of these catalysts to gasify carbon under high temperature steam conditions is that the metal agglomerates on the surface of the graphite which reduces the surface area of the metal thereby resulting in a concomitant reduction of catalytic activity. Inasmuch as the catalytic activity of such metals is an inverse function of the square of the square of the diameter of the particle size, smaller metal particles will result in much more rapid catalytic gasification of the carbon. Therefore, it would be a significant improvement to the art if one could gasify carbon with metal particles whose average size was less than about 100 Å in diameter, preferably less than 50 Å, more preferably below 25 Å and under conditions such that the metal particles will not agglomerate.

SUMMARY OF THE INVENTION

It has now been discovered that the disadvantages of the prior art are overcome by the present invention, which relates to catalytically gasifying carbon with steam in the presence of catalytic metal dispersed on the carbon wherein the average particle size of said dispersed metal is below about 100 Å in diameter, preferably below about 50 Å and still more preferably below about 25 Å, and under conditions such that the metal does not agglomerate. More particularly this invention is a process for catalytically gasifying carbon with steam in the presence of a catalytic metal comprising Ni, Co, Mo and mixtures thereof, said process comprising the steps of: (a) contacting a composite of said metal and graphite with an inert, hydrogen-containing atmosphere at a temperature ranging between about 800°-975° C. for a time sufficient for the metal to form a plurality of metal-containing channels in the graphite; (b) contacting said channeled composite formed in (a) with an inert hydrogen-containing atmosphere at a temperature of at least about 975° C. for a time sufficient for said metal in said channels to spread out and chemically wet at least a portion of the surface of said so-formed channels as a thin film of metal phase; (c) contacting said metal-wetted, channeled composite formed in (b)

with an oxidizing atmosphere at a temperature of at least about 800° C. to break up the metal phase film and form a dispersion of discrete particles of said metal on said graphite; and (d) contacting the dispersed metal-graphite composite formed in (c) with a steam atmosphere at a temperature of from about 800°-1,000° C. for a time sufficient for the metal to achieve the desired amount of gasification of the carbon. The particle size of the dispersed metal is controlled by the time, temperature and atmosphere employed in step (c). Preferred catalytic metals are Ni and Co. A particularly preferred metal is Ni.

Initial break-up of the metal phase film in step (c) results in a dispersion of discrete particles of metal having an average particle diameter below 25 Å. It is believed that initially the average metal particle diameter is below about 10 Å. However continued exposure to a mildly oxidizing atmosphere, such as steam, at elevated temperature causes the dispersed metal particles to agglomerate and grow in size.

It is essential to the process of this invention that the carbon be graphite or contain graphite such as a mixture of graphite with amorphous carbon. Illustrative but non-limiting examples of mixtures of graphite with other carbonaceous materials include asphalt, pitch, coke formed as a result of various hydrocarbon conversion reactions in petroleum refineries and petrochemical plants, etc., as well as coke formed on catalysts containing Ni, Co, Mo and mixtures thereof. As is well known to those skilled in the art, crystalline forms of carbon such as graphite have a basal plane or a-face (<1120> direction) and a plane perpendicular to the basal plane or c-face (<1010> direction). In the process of this invention, the catalytic metal creates channels in the c-face parallel to the a-face by catalytically gasifying the graphite with hydrogen. This increases the surface area of the c-face. It has been found that the metal will channel into the c-face surface and chemically wet the so-formed channels, but will not channel into the a-faces or basal planes.

As has heretofore been stated, catalytic metals that have been found to be useful for the process of this invention are Ni, Co, Mo and mixtures thereof. Nickel and cobalt are preferred and nickel is particularly preferred as the metal. It is understood, of course, that the process of this invention may start with a composite of the metal and graphite or graphite-containing material. Illustrative, but non-limiting examples include coke deposited on a metal surface containing one or more of said metals, such as coked steam cracker tubes, coked catalysts, etc. Alternatively, the metal may be added to the graphite or graphite-containing support by any convenient means known to those skilled in the art. Illustrative but nonlimiting examples include evaporating the metal onto the graphite in a vacuum, plasma or flame spraying the metal onto the support and various wet chemistry techniques employing metal precursors such as impregnation, incipient wetness, etc., followed by drying and contacting with a reducing atmosphere at elevated temperature to insure that the deposited metal is in the reduced, metallic form. Reducing the metal may be part of the heating step of the process wherein the composite is heated in a hydrogen atmosphere to form metal-containing channels in the graphite support. Metal precursors may be initially present on the graphite in the form of a metal salt or oxide such as carbonate, bicarbonate, sulfate, nitrate, etc., the main criterion

being that the metal precursor be capable of decomposing to or being reduced to the metal at a temperature below about 875° C. and preferably below about 800° C.

The metal-graphite composite must be heated in an inert, hydrogen-containing atmosphere at a temperature within the range of from about 800°-975° C. for a time sufficient for the metal to form a plurality of metal-containing channels in the graphite. By inert, hydrogen-containing atmosphere is meant an atmosphere that is net reducing to the metal or graphite and which will not adversely affect either the graphite support, the metal, or the gasification reaction. Enough hydrogen must be present to catalytically gasify and channel the graphite. The hydrogen may be a component of said atmosphere or it may be formed in-situ by using a mixture of, for example, steam and ethane and other mixtures of steam and saturated hydrocarbons, such as paraffins and saturated cyclic hydrocarbons. The temperature range for channeling is critical inasmuch as channels will not be formed at temperatures below about 800° C. At temperatures above about 975° C., in an inert, hydrogen-containing atmosphere, the metal will spread out and chemically wet the channels as a thin film at which point catalytic gasification and channeling cease. Channeling temperatures of from 800°-975° C. are preferred and particularly preferred are temperatures within the range of from about 800°-925° C.

When the metal channels into the c-face of the graphite, it does so by catalytically gasifying the carbon with hydrogen to form a gas such as methane. FIG. 1 schematically illustrates gasification and channeling of the graphite by a globule of nickel of about 500 Å in diameter. In a preferred embodiment of the invention, the metal-graphite composite will be heated within this temperature range in an inert, hydrogen-containing atmosphere for a time sufficient to achieve from about 5-20 wt. % gasification of the graphite support. Unless catalytic gasification of the graphite or graphite-amorphous carbon mixture is the desired result it is preferred that the total catalytic gasification of the graphite due to the channeling not exceed about 25 wt. % of the graphite. In practice, it has been found that the gasification rate of the graphite is roughly proportional to the concentration of metal thereon up to about 5 wt. % metal. As the amount of metal on the graphite exceeds about 5 wt. %, the gasification rate approaches a constant value.

After channeling of the graphite support has proceeded to the desired level, as evidenced by the amount of gasification of the graphite, the temperature is raised above about 975° C. at which point the metal in the channels spreads out and chemically wets the surface of the so-formed channels as a film of metal phase and catalytic gasification ceases. By chemical wetting it is meant that the metal wets and chemically bonds to the surface of the channels in the graphite. While not wishing to be held to any particular theory, it is believed that the metal chemically wets the channels as a film approximately one monolayer thick. The metal film exhibits strong interaction with the graphite support and is in itself a unique composition of matter inasmuch as it does not exhibit the properties of the bulk metal. Thus, the term "metal phase" refers to this unique film. In order for this metal-wetting to occur, it is important that the metal-graphite composite be in contact with an inert, hydrogen-containing atmosphere. This atmosphere must be net reducing with respect to both the metal and graphite support. A preferred temperature range for the wetting and metal phase film forming step will range

from about 975° to 1150° C., the upper limit being governed by noncatalytic gasification of the graphite which begins to occur at about 1200° C. in the presence of hydrogen. However, if necessary, one can exceed the upper limit of 1150° C. without adversely effecting the metal-wetted surface of the composite. One merely loses more graphite support.

The metal-wetted, channeled composite is then contacted with an oxidizing atmosphere, preferably a mild oxidizing atmosphere such as CO<sub>2</sub> or steam and most preferably steam, at a temperature of at least about 800° C. which breaks up the metal phase film in the channels into a highly dispersed form of metal which exists as discrete particles having an average diameter of less than 25 Å. It is believed that the average diameter of the metal particles is below about 10 Å when the metal film initially breaks up. However continued exposure of the dispersed-metal/graphite composite to a neutral (i.e., Ar, N<sub>2</sub>, Ne, He, etc.) atmosphere at higher temperatures of about 900° C. will cause these metal particles to agglomerate on the surface of the graphite and grow in size. The higher the temperature, the faster the agglomeration. If desired, particle sizes of 100 Å and even 500 Å or more in diameter can be achieved. This thus provides a novel and convenient way of achieving a wide range of average particle sizes having relatively narrow particle size distribution of the dispersed metal at any given particle size. It is understood, of course, that contacting the metal film/graphite composite with an oxidizing atmosphere to break up the film will result in at least a portion of the dispersed metal (i.e., at least a portion of the surface thereof) particles being in the oxide form which can then be reduced back to the metal by contact with a hydrogen-containing, net reducing atmosphere at a temperature below about 975° C. to avoid rewetting the graphite with the dispersed metal and concomitant film formation. This results in a much more active catalyst because of the greater metal area compared to conventional dispersions of metals, such as nickel on graphite, wherein the average particle diameter ranges from between about 50-1,000 Å and, more generally, between from about 100 to 250 Å.

In the final step of this process the so-formed dispersed metal/graphite composite may, if desired, again be contacted with a hydrogen containing atmosphere at a temperature of from about 800°-1,000° C. to cause catalytic gasification of the carbon via the same channeling mechanism as that used to initially form the channels. However, it is preferred to gasify the carbon in steam. Thus, the so-formed composite of highly dispersed metal on graphite is preferably contacted with steam at a temperature of from about 800°-1,000° C. for a time sufficient to achieve the desired amount of gasification. The amount of steam in the steam atmosphere may range from about 5% to 100% with the balance being an inert gas such as N<sub>2</sub>, Ar, He, Ne, Kr, etc. that does not react with either the metal or graphite. Interestingly, it has been found that the channeling rate in steam increases with decreasing catalytic metal particle size, whereas in hydrogen it increases with increasing particle size. In this step of the process gasification may, if desired, proceed until virtually complete gasification of the graphite or mixture of the graphite and amorphous carbon. Thus, it is known to those skilled in the art that a channeling and gasifying particle of catalyst metal will proceed into, channel and gasify amorphous carbon in contact with the graphite after the metal particle has channeled completely through the graphite.

However we have discovered that the metal will not chemically wet amorphous or non-graphitic carbon. Thus, even if it is desired to gasify primarily amorphous carbon, the amorphous carbon must contain some graphite at least initially in order to form the required metal/graphite composite and achieve the highly dispersed metal particles of small size thereon. By hydrogen-containing atmosphere it is again meant an atmosphere that is net reducing to both the catalytic metal and graphite and which contains enough hydrogen to achieve the desired carbon gasification.

#### BRIEF DESCRIPTION OF THE DRAWINGS

FIG. 1 is a schematic illustration of a globule of metal about 500 Å in diameter channeling into the c-face of graphite.

FIG. 2 is a schematic illustration of a globule or particle of channeling metal having the general shape of a hemispherical topped cylinder of diameter D.

FIG. 3 is a plot of experimental data showing the relative rate of graphite gasification in an inert, hydrogen-containing atmosphere as a function of nickel particle diameter at a given total quantity of nickel.

#### EXAMPLES

The invention will be more readily understood by reference to the examples below.

##### EXAMPLE 1

Spectrographically pure nickel (99.9% pure) was deposited onto transmission specimens of single crystals of graphite (Ticonderoga, New York State) as a monolayer film approximately one atom thick by evaporation from a heated tungsten filament at a residual pressure of  $5 \times 10^{-6}$  Torr. These nickel-containing specimens were placed in a controlled atmosphere electron microscope (CAEM) for the experimental work. Ethane 99.999% pure (Scientific Gas Products) was bubbled through water at 0° C. to generate a 40/1 ethane/water gas mixture which was then passed through the CAEM at a pressure of 1.0 Torr. As the nickel/graphite specimens were heated in the ethane/steam atmosphere in the CAEM, sporadic nucleation of the evaporated nickel film into small discrete particles was observed at a temperature of about 750° C. Those skilled in the art will know that the ethane/steam mixture formed hydrogen in-situ in the CAEM on contact with the nickel/graphite specimens. As the temperature was gradually raised to 890° C. particle nucleation and growth became more extensive and the first signs of catalytic attack were observed. This action was seen as the creation of very fine straight channels parallel to the a-face (<1120>) and perpendicular to the c-face produced by metal particles (50-150 Å diam.) which had collected at edges and steps on the surface. As the temperature was raised both the depth and size of particles propagating channels increased. At any given temperature it was apparent that the largest particles were producing channels at the fastest rates. Catalytic action increased in intensity until the temperature reached about 1000° C., when many of the narrower channels suddenly became devoid of catalyst particles at their head. This behavior became more generalized at 1050° C., extending to include even the larger particles (5,000 Å) and was identical in every respect to that observed for nickel/graphite specimens in a hydrogen atmosphere set forth in Example 4 below. Ultimately the channeling ceased as the nickel particles became completely disseminated.

Continued heating up to 1250° C. produced no further catalytic action or restoration of the original particles and only at the highest temperatures were indications of uncatalyzed gasification of graphite apparent. Discrete nickel particle formation was achieved again by treating these inactive specimens in oxygen at 850° C.

##### EXAMPLE 2

In this example, nickel/graphite specimens produced as in Example 1 were placed in the CAEM in the presence of pure (99.999%) oxygen at a pressure of 5 Torr. Nucleation of nickel particles was essentially complete at about 635° C. As the temperature was slowly raised, there was very little evidence of catalytic gasification. The experiment was concluded at 1150° C. due to vigorous, uncatalyzed gasification of the graphite which often resulted in specimen disintegration.

##### EXAMPLE 3

This experiment was similar to that in Examples 1 and 2, except that the atmosphere in the CAEM was 40/1 argon/steam at a pressure of 1 Torr. Thus, in this experiment as in that in Example 2, an oxidizing atmosphere was used in the CAEM. The results were similar to those in Example 2 except that catalytic gasification of the carbon ensued at about 935° C. with the nickel particles forming channels in the graphite parallel to the basal plane (<1120>). Uncatalyzed attack of the graphite became significant at about 1100° C.

##### EXAMPLE 4

This experiment was similar to that of Examples 1-3, except that the atmosphere in the CAEM was 1 Torr dry hydrogen (99.999% pure). Nickel particle nucleation commenced at about 755° C. with catalytic attack of the graphite commencing at about 845° C. which was seen as the development of fine channels parallel to the a-face of the graphite surface. As the temperature was raised, both the size and the number of channeling particles increased. The channels were up to 1500 Å in width, had many straight sections interrupted by changes in direction of 60° C. or 120° C., and were orientated parallel to (1120) directions. There were also examples of particles possessing hexagonal facets at the graphite-catalyst interface which were orientated parallel to (1010) directions.

On continued reaction it became evident that the channeling nickel particles were wetting the channels formed in the graphite thereby leaving material on the sides thereof. As a consequence, the nickel catalyst particles became smaller giving the channels a tapered appearance and, ultimately when all the catalyst was depleted, channels ceased to develop. The thickness of the nickel film formed on the surfaces of the channels was less than the 25 Å resolution of the CAEM. This wetting phenomenon, which started at 980° C., was essentially complete by the time the temperature had been raised to 1098° C. Continued heating in hydrogen up to 1250° C. produced no further catalytic action or restoration of the original particles and only at the highest temperature was it possible to detect signs of uncatalyzed attack. Subsequent cooling or heating in vacuo produced no change in specimen appearance, indicating that the metal-support interaction was very strong. It was significant that inactive particles remained static on the surface and showed less tendency to lose material during the reaction. If hydrogen was replaced by oxygen and the specimen reheated, then at 850° C. small

particles less than about 25 Å diameter started to reform along the edges of the original channels which were in the process of undergoing expansion due to uncatalyzed oxidation. This observation supported the idea that particle shrinkage in hydrogen was due to film formation along channel edges rather than volatilization. Eventually at 1065° C. in oxygen these particles proceeded to cut very fine channels emanating from the edges of the original channels. This behavior paralleled that found for Ni/graphite heated directly in oxygen.

#### EXAMPLE 5

This experiment was similar to those of Examples 1-4, except that the atmosphere in the CAEM was hydrogen/steam at a 40/1 ratio. The results were similar to those obtained in Example 4, except that channeling occurred at about 780° C. and uncatalyzed attack occurred at about 1150° C.

Thus, in oxidizing environments the major source of carbon gasification was due to uncatalyzed attack by the oxidizing atmosphere (Examples 2-3) whereas in the hydrogen-containing atmosphere, which was net reducing with respect to the nickel (Examples 1, 4 and 5) the carbon gasification was virtually completely catalytic. The most significant aspect of these examples resides in the discovery that, in an inert, hydrogen-containing atmosphere (net-reducing), the nickel spread out and wetted the so-formed channel surfaces and that if the so-formed nickel film was exposed to an oxidizing atmosphere (i.e., O<sub>2</sub> or H<sub>2</sub>O), discrete particles of nickel formed from the film on the channel surfaces and the catalytic gasification process could be repeated if one then switched back to an inert hydrogen-containing atmosphere. The cycle of channeling, wetting and redispersion of the nickel into discrete particles could be repeated indefinitely until there was virtually no graphite left.

#### EXAMPLE 6

This experiment was identical to that of Example 1, except that the atmosphere in the CAEM was ethane/hydrogen/steam in a ratio of approximately 38/2/1, respectively. Nickel particle nucleation occurred at about 750° C., but was much crisper than that in Example 1 and channeling occurred at about 845° C. The presence of 5% hydrogen in the ethane/steam mixture of Example 1 resulted in a five-fold increase in the rate of the nickel catalyzed gasification of the graphite.

#### EXAMPLE 7

This example demonstrates the unusual and unique hydrogen chemisorption properties of the wetted nickel film on the channel surfaces of the graphite. Nickel on Grafoil specimens were prepared using an incipient wetness technique. 5 mm disks of Grafoil were soaked in a solution of nickel acetate in methanol for one-half hour at 80° C. after which the Grafoil disks were dried for eight hours at 120° C. and washed with methanol to remove the excess nickel salt to produce a nickel/Grafoil precursor. The unreduced nickel content of this precursor material was 2.7 wt. percent. This precursor was reduced for two hours at 600° C. in pure hydrogen to produce nickel/Grafoil specimens. Specific details of the subsequent experiments are given in Tables 1-3 which are summarized below.

Following reduction at 600° C., the nickel/Grafoil specimens adsorbed (per gram) 0.080 cc of hydrogen, of which 0.048 cc was reversibly adsorbed, at an equilib-

rium hydrogen pressure of 0.26 atm. Under the same conditions, but following an additional treatment in hydrogen at 1100° C. for one hour, the nickel/Grafoil composite did not show any hydrogen chemisorption capacity which indicates a modification in the hydrogen chemisorption properties of nickel in the new state produced by the latter treatment. When this material was steamed at 1000° C. in a H<sub>2</sub>O:He stream (1:40) for one to two hours; the hydrogen capacity was partially restored as 0.043 cc of hydrogen could be chemisorbed. By further rereduction at 600° C. for 0.5 hours, the latter value was increased to 0.052 cc of hydrogen per gram of catalyst. It was then concluded that steaming the modified nickel/Grafoil composite restored the original chemisorption properties of the nickel.

This example demonstrates that:

- o: treatment in hydrogen at 1000°-1110° C. of nickel on graphite (Grafoil) leads to a new chemical state of nickel in which the metal does not show its usual hydrogen chemisorption properties,
- o: the new chemical state of nickel on graphite (Grafoil) that can be prepared by the above treatment can be broken to regenerate the nickel film as small nickel particles which chemisorb hydrogen.

Additional experiments employing ferromagnetic resonance studies of the nickel/Grafoil specimens supported the hydrogen chemisorption studies and reinforced the conclusions that a film-like nickel phase was formed by wetting in the channels and that this phase strongly interacts with the Grafoil support and contains very little dissolved carbon.

#### EXAMPLE 8

This example demonstrates the great increase in the overall rate of gasification of graphite that is achieved when a large particle of metal is redispersed into a number of smaller particles.

The following example is designated to demonstrate the enhancement in the overall rate of carbon gasification realized when one redisperses a large catalyst particle into numerous smaller components.

The catalytic effect of two particles, (a) 80 Å in diameter and (b) 800 Å in diameter, which gasify carbon by the channeling mode is examined using the following mathematical procedure:

##### (i) Computation of the Particle Volumes

During channel formation, electron microscopy has revealed that channeling particles assume a shape which is best approximated by a cylinder of diameter D and height W surmounted by a hemisphere of diameter D, as depicted in FIG. 2. The cylindrical portion of the particle is embedded in the channel, and the hemispherical portion projects from the surface. The volume of such a particle is given by:

$$V = \frac{\pi D^2}{4} W + \frac{2}{3} \frac{\pi D^3}{8} \quad (1)$$

Experimental evidence obtained from a shadowing procedure indicate that (W/D)=0.25, which reduces to

$$V = \frac{7}{48} \pi D^3 \quad (2)$$

For a particle where D=8 nm, V=2.35×10<sup>2</sup> nm<sup>3</sup> and where D=80 nm, V=2.35×10<sup>5</sup> nm<sup>3</sup>. We can therefore

generate 1000 particles ( $D=8$  nm) from 1 particle ( $D=80$  nm).

(ii) Calculation of Amount of Carbon Gasified as a Function of Catalyst Particle Size

The number of moles of carbon gasified per second,  $(dn/dt)$  is given by:

$$\frac{dn}{dt} = \frac{IDW\rho}{M} \quad (3)$$

where

$1$  is the rate of channel propagation

$D$  is the particle diameter

$W$  is the depth of the channel

$\rho$  is the density of graphite,  $2.25$  g  $cm^{-3}$

$M$  is the atomic weight of carbon,  $12$

The experimentally determined relationship between rate of channel propagation and nickel particle size for gasification of carbon in steam at  $1000^\circ C.$  is given in FIG. 3 from nickel/graphite specimens prepared following the procedure in Example 1.

This data was obtained from direct observation of the catalytic reaction using controlled atmosphere electron microscopy. The changes in appearance of the specimen are continuously recorded on video-tape and this information is subsequently transferred to  $16$  mm cine film. Detailed kinetic analysis is performed from frame by frame projection of the movie. In this particular case one measures the linear increase in channel length as a function of time; from such measurements it is simple operation to calculate the rate of reaction of a given sized particle. Since the depths of channels vary from particle to particle, comparisons such as that given in FIG. 3 are made from particles channeling at a similar depth to each other. This aspect is determined from the difference in contrast in the image between the channel and the surrounding unattacked graphite. Thus the only variables in the measurements plotted in FIG. 3 are the particle sizes and the linear propagation rate of the channels.

From this data we find that the rate of channels propagated by  $80$  nm diameter particles is  $3.75$  nm  $s^{-1}$ , and that by  $8$  nm diameter particles is  $12.2$  nm  $s^{-1}$ . Assuming that  $W$  is  $(D/4)$ , we can calculate the number of moles of carbon gasified per sec. by each of these particles by substitution of the numerical values into equation 3. For  $80$  nm diam. particles,  $(dn/dt)=1.125 \times 10^{-18}$  moles  $s^{-1}$  and for  $8$  nm diam. particles,  $(dn/dt)=3.66 \times 10^{-20}$  mole  $s^{-1}$ . However, as shown previously one  $80$  nm diam. particle can create  $1000$ ,  $8$  nm diam. particles, and in this case the total number of moles of carbon gasified per second would be  $3.66 \times 10^{-17}$  moles  $s^{-1}$ , i.e. this would result in a net increase in carbon gasification rate of  $32.5$  times that generated by the one larger particle.

TABLE 1  
TREATMENTS AND HYDROGEN CHEMISORPTIONS  
ON NICKEL/GRAPHOIL

|     | Treatment              | Temperature<br>( $^\circ C.$ ) | Measurements |
|-----|------------------------|--------------------------------|--------------|
| (A) | Reduction in $H_2$     | 600                            |              |
|     | Evacuation             | 550                            |              |
|     | Evacuation             | 25                             |              |
|     | Chemisorption of $H_2$ | 25                             |              |
|     | Treatment in $H_2$     | 1095                           | $C_1, C_2$   |
|     | Evacuation             | 550                            |              |
|     | Evacuation             | 25                             |              |

TABLE 1-continued

| TREATMENTS AND HYDROGEN CHEMISORPTIONS<br>ON NICKEL/GRAPHOIL |                        |                                |              |
|--------------------------------------------------------------|------------------------|--------------------------------|--------------|
|                                                              | Treatment              | Temperature<br>( $^\circ C.$ ) | Measurements |
| 5                                                            | Chemisorption of $H_2$ | 25                             | $C_3, C_4$   |
| 10                                                           | Treatment in $H_2$     | 1000                           |              |
|                                                              | Evacuation             | 500                            |              |
|                                                              | Desorption             | 1000                           | $D_1$        |
|                                                              | Evacuation             | 950                            |              |
|                                                              | Evacuation             | 25                             |              |
| 15                                                           | Chemisorption of $H_2$ | 25                             | $C_5$        |
|                                                              | Steaming               | 800                            |              |
|                                                              | Purging in $He$        | 300                            |              |
|                                                              | Evacuation             | 25                             |              |
|                                                              | Chemisorption of $H_2$ | 25                             | $C_6$        |
|                                                              | Steaming               | 1000                           |              |
|                                                              | (c)                    | —                              |              |
|                                                              | Chemisorption of $H_2$ | 25                             | $C_7$        |
|                                                              | a + b                  | —                              |              |
|                                                              | Chemisorption of $H_2$ | 25                             | $C_3$        |
|                                                              | Steaming               | 1,000                          |              |
|                                                              | (c)                    | —                              |              |
|                                                              | Chemisorption of $H_2$ | 25                             | $C_6$        |
|                                                              | Treatment in $H_2$     | 600                            |              |
|                                                              | Evacuation             | 25                             |              |
|                                                              | Chemisorption of $H_2$ | 25                             | $C_8$        |

TABLE 2

CHEMISORPTION OF HYDROGEN ON  
NICKEL/GRAPHOIL CATALYSTS

| Run | Treatment <sup>(a)</sup>                                                   | Volume $H_2$<br>Adsorbed <sup>(b)</sup> |
|-----|----------------------------------------------------------------------------|-----------------------------------------|
| 30  | 1. $C_1$ Reduced $600^\circ C.$ , total                                    | 0.080                                   |
|     | $C_2$ Reduced $600^\circ C.$ , reversible                                  | 0.048                                   |
|     | $C_3$ Treated $1095^\circ C.$ in $H_2$ , 2 hrs                             | 0.020                                   |
|     | $C_4$ Evacuated $25^\circ C.$ , following $C_3$                            | 0.023                                   |
|     | $C_5$ Evacuated $1000^\circ C.$                                            | 0.0                                     |
|     | $C_6$ Steaming $800^\circ C.$                                              | 0.0                                     |
|     | $C_7$ Steaming $100^\circ C.$                                              | 0.042                                   |
| 35  | 2. $C'_3$ Reduced $600^\circ C.$ , treated $1000^\circ C.$ in $H_2$ , 1 hr | 0.0                                     |
|     | $C'_6$ Steamed $100^\circ C.$ , 1 hr                                       | 0.0425                                  |
|     | $C'_7$ Reduced $600^\circ C.$                                              | 0.0525                                  |

(a) See Table 1 for details

(b) Value at an equilibrium pressure of  $200$  Torr. cc  $H_2$  STP/gram of catalyst.

TABLE 3

X-RAY DIFFRACTION AND CHEMISORPTION DATA  
ON TREATED NI/GRAPHOIL SPECIMENS

| Treatment                                                                                                                               | $H_2$ Chemisorption<br>and X-ray                                                   |
|-----------------------------------------------------------------------------------------------------------------------------------------|------------------------------------------------------------------------------------|
| 1. Reduced at $600^\circ C.$                                                                                                            | Large particles and normal $H_2$ Chemisorption                                     |
| 2. Reduced at $600^\circ C.$ , treated in $H_2$ at $1000^\circ C.$ , evacuated at $950^\circ C.$ followed by steaming at $800^\circ C.$ | Smaller particles, but poor $H_2$ chemisorption, about zero (see $C_6$ - Table 2). |

What is claimed is:

1. A process for catalytically gasifying carbon with steam in the presence of a catalytic metal comprising Ni, Co, Mo and mixtures thereof, said process comprising the steps of:

- contacting a composite of said metal and graphite with an inert, hydrogen-containing atmosphere at a temperature ranging between about  $800^\circ$ – $975^\circ C.$  for a time sufficient for the metal to form a plurality of metal-containing channels in the graphite;
- contacting said channeled composite formed in (a) with an inert hydrogen-containing atmosphere at a temperature of at least about  $975^\circ C.$  for a time

- sufficient for said metal in said channels to spread out and chemically wet at least a portion of the surface of said channels;
- (c) contacting said metal-wetted, channeled composite formed in (b) with an oxidizing atmosphere at a temperature of at least about 800° C. to form a dispersion of discrete particles of said metal on said graphite; and
- (d) contacting the dispersed metal/graphite composite formed in (c) with steam at a temperature of at least about 800° C. for a time sufficient for the metal to achieve the desired amount of gasification of the carbon.

2. The process of claim 1 wherein the average diameter of the metal particles formed in (c) is below about 100 Å.

3. The process of claim 2 wherein said catalytic metal particles formed in (c) have an average diameter below about 25 Å.

4. The process of claim 3 wherein the contacting temperature in step (d) ranges from about 800°-1,000° C.

5. The process of claim 4 wherein in step (c) the contacting atmosphere is mildly oxidizing.

6. The process of claim 5 wherein said catalytic metal is Ni, Mo, and mixtures thereof.

7. The process of claim 6, wherein said oxidizing atmosphere in (c) comprises from 5% to 100% steam.

10

20

25

30

8. The process of claim 7 wherein said catalytic metal is Ni.

9. A process for catalytically gasifying carbon with hydrogen in the presence of a catalytic metal comprising Ni, Co, Mo and mixtures thereof, said process comprising steps of:

- (a) contacting a composite of said metal and graphite with an inert, hydrogen-containing atmosphere at a temperature ranging between about 800°-975° C. for a time sufficient for the metal to form a plurality of metal-containing channels in the graphite;
- (b) contacting said channeled composite formed in (a) with an inert hydrogen-containing atmosphere at a temperature of at least about 975° C. for a time sufficient for said metal in said channels to spread out and chemically wet at least a portion of the surface of said channels;
- (c) contacting said metal-wetted, channeled composite formed in (b) with an oxidizing atmosphere at a temperature of at least about 800° C. to form a dispersion of discrete particles of said metal on said graphite; and
- (d) contacting the dispersed metal/graphite composite formed in (c) with an inert, hydrogen-containing atmosphere at a temperature ranging between about 800°-1000° C. for a time sufficient for the metal to achieve the desired amount of gasification of the carbon.

\* \* \* \* \*

35

40

45

50

55

60

65